# EUROPEAN PATENT SPECIFICATION

(11) **EP 0 504 154 B1**
(45) Date of publication and mention of the grant of the patent: **15.12.1993**
(21) Application number: 90916275.2
(22) Date of filing: 14.11.1990
(51) Int. Cl.: G03C 7/36, G03C 1/34, C07C 39/16

(54) **PHOTOGRAPHIC SILVER HALIDE MATERIALS**
PHOTOGRAPHISCHES SILBERHALOGENIDMATERIAL
MATERIAUX PHOTOGRAPHIQUES A BASE D'HALOGENURE D'ARGENT

(30) Priority: 06.12.1989 GB 8927563
(43) Date of publication of application: 23.09.1992
(73) Proprietor: KODAK LIMITED, Harrow, Middlesex HA1 4TY (GB); EASTMAN KODAK COMPANY, Rochester, New York 14650-2201 (US)
(72) Inventor: LEYSHON, Llewellyn James, Watford, Hertfordshire WD1 3HW (GB); GODDARD, John Demita, Pinner, Middlesex HA5 3EW (GB)
(74) Representative: Baron, Paul Alexander Clifford
(86) International application number: EP9001963
(87) International publication number: WO9108515

(56) References cited:
- EP-A- 0 230 659
- EP-A- 0 231 832
- EP-A- 0 256 531
- US-A- 3 933 501
- US-A- 4 782 011
- US-A- 4 783 397
- Research Disclosure No.17 643(12.78)
- British Journal of Photography annual 1986,pages 37 and 38
- Kubo:Toward the New Age of Colour Print,Shashin Koggo,vol.44,No.8,08.86,pages 95-98 and English translation

## Description

This invention relates to photographic silver halide materials.

European Patent Specification 0 246 766 (or US Patent 4 782 011) describes the stabilisation of photographic dye images using a bisphenol derivative having two linked phenol rings, one of the phenolic hydroxy groups being substituted and at least one of the phenol rings being substituted.

We have now found that the same bisphenol compounds will, in silver chloride emulsions suitable for processing in a colour developer free of benzyl alcohol, ensure that the performance of a certain class of yellow couplers is maximised.

According to the present invention therefore there is provided a method of increasing the Dₘₐₓ and gamma and decreasing the Dₘᵢₙ of the yellow dye image formed in a photosensitive photographic colour material comprising a support bearing a silver halide emulsion layer, the halide content of which is at least 85% chloride, and which contains in or adjacent said silver halide layer a ballasted yellow coupler of the general formula:
wherein
L¹ is -NHSO₂, -SO₂NH-, -OCO-, -COO-, -OSO₂- or -SO₂O-,
R¹ is halogen or an alkyloxy group of 1-4 carbon atoms,
R² is a substituted or unsubstituted alkyl of a substituted or unsubstituted aryl group of sufficient size and configuration to render the coupler non-diffusible in the photographic material, and
X is a halogen, aryloxy, arylthio or heterocyclic coupling-off group
upon imagewise exposure and colour processing thereof including the step of colour development in the absence of benzyl alcohol by incorporating in the layer containing said coupler a bisphenol derivative having two linked phenol rings, one of the phenolic hydroxy groups being substituted by a blocking group and at least one of the phenol rings being substituted.

The photographic materials improved by the method of the present invention containing the combination of said stabilisers and said yellow image dye-forming couplers show maximised coupler performance as measured by higher Dₘₐₓ and/or gamma and reduced Dₘᵢₙ of the dye image. Other known dye image stabilisers do not have this effect. Dye image stabilisation is also superior to that obtained with other known stabilisers.

The ballasting groups R² may include alkyl and/or aryl moieties optionally linked by ether or ester groups. Examples of such groups which may be employed are:

The coupling-off group X may be chlorine a heterocyclic group or an aryloxy or arylthio group optionally substituted with alkyl or arylsulphonyl, alkylsulphonamido, or alkoxycarbonyl groups which themselves are optionally substituted. Preferred coupling-off groups are phenoxy groups containing electron-withdrawing substituents at the ortho- and/or para positions, especially at the para- and one ortho-position. In addition, ionisable substituents are also beneficial. Examples of coupling-off groups that may be used are the following:
(a)
(b)
(c)
(d)
(e)
(f)
(g)
(h)
(i)
(j)

   -Cl
(k)

Examples of couplers according to the present invention are listed in the following Table.

A preferred group of bisphenol compounds are known dye image stabilisers represented by the following general formula
wherein
A is a blocking group such as alkyl e.g. methyl, ethyl, propyl or butyl; cycloalkyl e.g. cyclohexyl; alkenyl; aryl e.g. phenyl; acyl e.g. acetyl or benzoyl; alkylsulphonyl or arylsulphonyl;
L is a single bond or a linking group such as alkylene e.g. methylene; alkylidene e.g. butylidene or 3,5,5,-trimethylhexylidene; a heteroatom e.g. oxygen or sulphur; or sulphonyl; and,
each R independently represents one or more substituents each independently selected from alkyl, alkoxy, alkenyl, cycloalkyl, or aryl; or each R independently represents the atoms necessary to complete with the benzene ring to which it is attached a fused polycyclic aromatic ring structure;
all the above mentioned alkyl, cycloalkyl, alkylene, alkenyl, acyl and aryl groups being optionally substituted.

Particularly preferred bisphenols are represented by the general formula
wherein
A and L are as defined above; and,
R³, R⁴, R⁵ and R⁶ each independently represent substituted or unsubstituted alkyl, alkenyl, cycloalkyl or aryl. Preferably, R³ and R⁴ are identical and R⁵ and R⁶ are identical.

Alkylidene bisphenols represent a preferred group of stabilizers in which the linking group L may be -(CR⁷R⁸)ₙ- wherein each of R⁷ and R⁸ independently is hydrogen or optionally substituted alkyl, cycloalkyl, alkenyl or aryl and n is an integer from 1 to 10, preferably 1 to 3, most preferably 1.

Specific examples of a bisphenol suitable for use in the present invention are as follows:
Other examples are listed in European Specification 0 246 766.

The silver halide preferably comprises at least 95% chloride and is preferably substantially pure silver chloride.

Typically both the coupler and the bisphenol derivative are dissolved in a coupler solvent and this solution is dispersed in an aqueous gelatin solution. Examples of coupler solvents that may be used are dibutyl phthalate, tricresyl phosphate, diethyl lauramide and 2,4-di-tertiary-amylphenol. In addition an auxiliary coupler solvent may also be used, for example ethyl acetate, cyclohexanone, and 2-(2-butoxy-ethoxy)ethyl acetate, which are removed from the dispersion before incorporation into the photographic material.

The photographic elements can be single colour elements or multicolour elements. In a multicolour element, the yellow dye-forming couplers of this invention would usually be associated with a blue-sensitive emulsion, although they could be associated with an emulsion sensitised to a different region of the spectrum, or with a panchromatically sensitised, orthochromatically sensitised or unsensitised emulsion. Multicolour elements contain dye image-forming units sensitive to each of the three primary regions of the spectrum. Each unit can be comprised of a single emulsion layer or of multiple emulsion layers sensitive to a given region of the spectrum. The layers of the elements, including the layers of the image-forming units, can be arranged in various orders as known in the art.

A typical multicolour photographic element comprises a support bearing a yellow dye image-forming unit comprised of at least one blue-sensitive silver halide emulsion layer having associated therewith at least one yellow dye-forming coupler and magenta and cyan dye image-forming units comprising at least one green- or red-sensitive silver halide emulsion layer having associated therewith at least one magenta or cyan dye-forming coupler respectively. The element can contain additional layers, such as filter layers.

In the following discussion of suitable materials for use in the emulsions and elements of this invention, reference will be made to Research Disclosure, December 1978, Item 17643, published by Industrial Opportunities Ltd., The Old Harbourmaster's, 8 North Street, Emsworth, Hants PO10 7DD, U.K. This publication will be identified hereafter as "Research Disclosure".

The silver halide emulsion employed in the elements improved by this invention can be either negative-working or positive-working. Suitable emulsions and their preparation are described in Research Disclosure Sections I and II and the publications cited therein. Suitable vehicles for the emulsion layers and other layers of elements of this invention are described in Research Disclosure Section IX and the publications cited therein.

In addition to the couplers of this invention, the elements can include additional couplers as described in Research Disclosure Section VII, paragraphs D, E, F and G and the publications cited therein. The couplers of this invention and any additional couplers can be incorporated in the elements and emulsions as described in Research Disclosures of Section VII, paragraph C and the publications cited therein.

The photographic elements or individual layers thereof, can contain brighteners (see Research Disclosure Section V), antifoggants and stabilisers (see Research Disclosure Section VI), antistain agents and image dye stabiliser (see Research Disclosure Section VII, paragraphs I and J), light absorbing and scattering materials (see Research Disclosure Section VIII), hardeners (see Research Disclosure Section XII, plasticisers and lubricants (see Research Disclosure Section XIII), matting agents (see Research Disclosure Section XVI) and development modifiers (see Research Disclosure Section XXI).

The photographic elements can be coated on a variety of supports as described in Research Disclosure Section XVII and the references described therein.

Photographic elements can be exposed to actinic radiation, typically in the visible region of the spectrum, to form a latent image as described in Research Disclosure Section XVIII and then processed to form a visible dye image as described in Research Disclosure Section XIX. Processing to form a visible dye image includes the step of contacting the elements with a colour developing agent to reduce developable silver halide and oxidise the colour developing agent. Oxidised colour developing agent in turn reacts with the coupler to yield a dye.

Preferred colour developing agents are p-phenylene diamines. Especially preferred are 4-amino-3-methyl-N,N-diethylaniline hydrochloride, 4-amino-3-methyl-N-ethyl-N-β-(methylanesulphonamido)ethylaniline sulphate hydrate, 4-amino-3-methyl-N-ethyl-N-β-(methanesulphonamide)ethyl-N,N-diethylaniline hydrochloride and 4-amino-N-ethyl-N-(2-methoxyethyl)-m-toluidine di-p-toluene sulphonate.

With negative-working silver halide emulsions this processing step leads to a negative image. To obtain a positive (or reversal) image, this step can be preceded by development with a non-chromagenic developing agent to develop exposed silver halide, but not form dye, and then uniform fogging of the elements to render unexposed silver halide developable. Alternatively, a direct positive emulsion can be employed to obtain a positive image.

Development is followed by the conventional steps of bleaching, fixing, or bleach-fixing, to remove silver and silver halide, washing and drying.

The invention is illustrated by the following Examples.

### Example 1

Two dispersions of Coupler (1) in gelatin, with and without added Compound (1), were prepared by ultrasonic agitation (Dawe Instruments "Soniprobe"). Details of the method are given below:
(i) Oil Solution:
   - Coupler (1): 3.28g
   - dibutyl phthalate: 0.82g
   - 2-(2-butoxyethoxy)ethyl acetate: 0.82g
   - Compound (1): 1.64g
(ii) Gel Solution:

The components of the oil solution were heated together at 120°C to effect solution. A small quantity of ethyl acetate (O.5g) was added to help this process and this was evaporated off before continuing. The gelatin mixture, melted at 60°C, was added to the hot oil and the mixture agitated with the ultrasonic probe for 4 minutes and chilled.

A similar dispersion of a check Coupler (A) (identified below) without stabiliser was also prepared.

The Coupler (1) dispersions were coated with a blue-sensitive AgCℓ emulsion to give coatings of the following structure:

The Coupler (A) dispersion was coated similarly except that the coupler coverage was increased to 0.753g per square metre.

The coatings were wedge-exposed and developer using RA4 processing solutions. Sensitometric parameters were recorded and the sample strips were then faded for 10 days through a UV filter in front of a high intensity light source (Xenon Arc, 50 Klux). The loss of dye density from an initial value of 1.0 was recorded. The results are shown in the table below:

The gamma, or contrast, values shown in the table can be taken to represent the photographic activity of the coatings. It is clear that the presence of Compound (1) improved the performance Coupler (1), and that both Coupler (1) coatings were superior to the Coupler (A) check, notwithstanding the 28% higher coverage of the check coupler.
Coupler (A) has the formula:

The recorded fades show that the presence of the stabiliser produces a substantial improvement in the light stability of the coupler (1) image dye, to the extent that it surpasses that of the (unstabilised) check.

### Example 2

Further Coupler (1) dispersions were prepared and coated as in Example 1, containing, respectively, no stabiliser, and various stabilisers including some outside the present invention. Compared with Example 1, the coating coverages were reduced to 0.382g per square metre coupler and 0.17g per square metre Ag.

The coatings were evaluated in the same manner as in Example 1 and the Table below shows the results.

The gamma values in the table confirm the sensitometric benefit of Compound (1) and show similar behaviour for its analogue, Compound (2). In contrast, both of the comparison stabilisers,
Compound (A):
and Compound (B) (Irgaperm 1994 (trade name of Ciba-Geigy)) were detrimental to sensitometry. Furthermore, these stabilisers were found to be significantly less effective than the two materials of this invention in reducing the fade of the image.

### Example 3

Coatings were made and tested as described in Example 1 using the couplers indicated below with silver and coupler coverages at 0.465 g/m² and 0.215 g/m² respectively. The results were as follows.

Improvements are seen not only in fade results but both D_{min,} Dₘₐₓ and, for Coupler (6), gamma as well.

## Claims

1. A method of increasing the Dₘₐₓ and gamma and decreasing the Dₘᵢₙ of the yellow dye image formed in a photosensitive photographic colour material comprising a support bearing a silver halide emulsion layer, the halide content of which is at least 85% chloride, and which contains in or adjacent said silver halide layer:
a ballasted yellow coupler of the general formula: wherein
L¹ is -NHSO₂, -SO₂NH-, -OCO-, -COO-, -OSO₂- or -SO₂O-,
R¹ is halogen or an alkyloxy group of 1-4 carbon atoms,
R² is a substituted or unsubstituted alkyl or a substituted or unsubstituted aryl group of sufficient size and configuration to render the coupler non-diffusible in the photographic material, and
X is a halogen, aryloxy, arylthio or heterocyclic coupling-off group
upon imagewise exposure and colour processing thereof including the step of colour development in the absence of benzyl alcohol. by incorporating in the layer containing said coupler a bisphenol derivative having two linked phenol rings, one of the phenolic hydroxy groups being substituted by a blocking group and at least one of the phenol rings being substituted.

2. A method as claimed in claim 1 wherein the group R² comprises a group:

3. A method as claimed in claim 1 or 2 in which the group R¹ is chloro or methoxy.

4. A method as claimed in any of claims 1-3 in which the coupling off group X is one of the following:
(a)
(b)
(c)
(d)
(e)
(f)
(g) or
(h)
(i)
(j)
-Cl
(k)

5. A method as claimed in any of claims 1-4 in which the bisphenol derivative has the general formula: wherein
A is a blocking group such as alkyl e.g. methyl, ethyl, propyl or butyl; cycloalkyl e.g. cyclohexyl; alkenyl; aryl e.g. phenyl; acyl e.g. acetyl or benzoyl; alkylsulphonyl or arylsulphonyl;
L is a single bond or a linking group such as alkylene e.g. methylene; alkylidene e.g. butylidene or 3,5,5,-trimethylhexylidene; a heteroatom e.g. oxygen or sulphur; or sulphonyl; and,
each R independently represents one or more substituents each independently selected from alkyl, alkoxy, alkenyl, cycloalkyl, or aryl; or each R independently represents the atoms necessary to complete with the benzene ring to which it is attached a fused polycyclic aromatic ring structure;
all the above mentioned alkyl, cycloalkyl, alkylene, alkenyl, acyl and aryl groups being optionally substituted.

6. A method as claimed in any of claims 1-5 in which the bisphenol derivative has the general formula: wherein
A and L are as defined in claim 5; and,
R³, R⁴ , R⁵ and R⁶ each independently represents substituted or unsubstituted alkyl, alkenyl, cycloalkyl or aryl. Preferably, R³ and R⁴ are identical and R⁵ and R⁶ are identical.
Alkylidene bisphenols represent a preferred group of stabilizers in which the linking group L may be -(CR⁷R⁸)ₙ- wherein each of R⁷ and R⁸ independently is hydrogen or optionally substituted alkyl, cycloalkyl, alkenyl or aryl and n is an integer from 1 to 10, preferably 1 to 3, most preferably 1.

7. A method as claimed in any of claims 1-6 in which the bisphenol compound has one of the formulae: and

8. A method as claimed in any of claims 1-7 in which the coupler is one of those listed in the following Table: in which the groups (f), (c), (g) and (k) are as defined in Claim 4.

9. A method as claimed in any of claims 1-8 wherein the photographic material is a multicolour photographic element comprising a support bearing a yellow dye image-forming unit comprised of at least one blue-sensitive silver halide emulsion layer having associated therewith at least one coupler and one blocked bis-phenol as defined in any of claims 1 - 8 and magenta and cyan dye image-forming units comprising at least one green- or red-sensitive silver halide emulsion layer having associated therewith at least one magenta or cyan dye-forming coupler respectively.

## Patentansprüche

1. Verfahren zur Erhöhung von Dₘₐₓ und Gamma sowie zur Verminderung von Dₘᵢₙ des gelben Farbstoffbildes, das in einem photosensitiven photographischen Farbmaterial erzeugt worden ist, das aufweist einen Träger, auf dem sich eine Silberhalogenidemulsionsschicht befindet, wobei der Halogenidgehalt derselben bei mindestens 85 % Chlorid liegt und das in oder benachbart zur Silberhalogenidschicht einen eine Ballastgruppe aufweisenden gelben Kuppler der allgemeinen Formel aufweist: worin bedeuten: L¹ eine Gruppe der Formeln -NHSO₂-, -SO₂NH-, -OCO-, -COO-, -OSO₂- oder -SO₂O-,
R¹ ein Halogenatom oder eine Alkoxygruppe mit 1 bis 4 Kohlenstoffatomen,
R² eine substituierte oder unsubstituierte Alkyl- oder eine substituierte oder unsubstituierte Arylgruppe einer solchen Größe und Konfiguration um den Kuppler in dem photographischen Material nicht-diffundierend zu machen, und
X eine ab-kuppelnde Halogen-, Aryloxy-, Arylthio- oder heterocyclische Gruppe,
das die bildweise Exponierung und Farbentwicklung umfaßt einschließlich der Stufe der Farbentwicklung in Abwesenheit von Benzylalkohol, durch Einverleiben eines Bisphenolderivates mit zwei miteinander verbundenen Phenolringen, wobei eine der phenolischen Hydroxygruppen substituiert ist durch eine blokkierende Gruppe und wobei mindestens einer der Phenolringe substituiert ist, in die Schicht, die den Kuppler enthält.

2. Verfahren nach Anspruch 1, bei dem die Gruppe R² eine Gruppe der folgenden Formeln umfaßt:

3. Verfahren nach Anspruch 1 oder 2, bei dem die Gruppe R¹ eine Chlor- oder Methoxygruppe ist.

4. Verfahren nach einem der Ansprüche 1 bis 3, in dem die abkuppelnde Gruppe X eine Gruppe der folgenden Formeln ist:
(a)
(b)
(c)
(d)
(e)
(f)
(g)
(h)
(i)
(j)
-Cl
(k)

5. Verfahren nach einem der Ansprüche 1 bis 4, bei dem das Bisphenolderivat der folgenden allgemeinen Formel entspricht: worin bedeuten:
A eine blockierende Gruppe, wie z. B. eine Alkylgruppe, z. B. Methyl, Ethyl, Propyl oder Butyl; eine Cycloalkylgruppe, z. B. Cyclohexyl; eine Alkenylgruppe; eine Arylgruppe, z. B. Phenyl; eine Acylgruppe, z. B. Acetyl oder Benzoyl; Alkylsulphonyl oder Arylsulphonyl;
L eine einzelne Bindung oder eine verbindende Gruppe, z. B. eine Alkylengruppe, z. B. Methylen; eine Alkylidengruppe, z. B. Butyliden oder 3,5,5-Trimethylhexyliden; ein Heteroatom, z. B. Sauerstoff oder Schwefel; oder eine Sulphonylgruppe; und
R jeweils unabhängig voneinander einen oder mehrere Substituenten, jeweils unabhängig voneinander ausgewählt aus Alkyl, Alkoxy, Alkenyl, Cycloalkyl oder Aryl; oder R unabhängig voneinander die Atome, die gemeinsam mit dem Benzolring, an den R gebunden ist, eine ankondensierte polycyclische aromatische Ringstruktur bilden;
wobei gilt, daß sämtliche der angegebenen Alkyl-, Cycloalkyl-, Alkylen-, Alkenyl-, Acyl- und Arylgruppen gegebenenfalls substituiert sein können.

6. Verfahren nach einem der Ansprüche 1 bis 5, bei dem das Bisphenolderivat der allgemeinen Formel: entspricht, worin bedeuten:
A und L Reste der in Anspruch 5 angegebenen Bedeutung; und
R³, R⁴, R⁵ und R⁶ jeweils unabhängig voneinander substituierte oder unsubstituierte Alkyl-, Alkenyl-, Cycloalkyl- oder Aryl-gruppen, wobei R³ und R⁴ vorzugsweise identisch sind und R⁵ und R⁶ identisch sind, wobei
Alkylidenbisphenole eine bevorzugte Gruppe von Stabilisatoren darstellen, in denen die verbindende Gruppe L der Formel (CR⁷R⁸)ₙ- entsprechen kann, worin R⁷ und R⁸ jeweils unabhängig voneinander stehen für Wasserstoff oder gegebenenfalls substituierte Alkyl-, Cycloalkyl-, Alkenyl- oder Arylgruppen und worin n eine Zahl von 1 bis 10, vorzugsweise 1 bis 3 und insbesondere 1 ist.

7. Verfahren nach einem der Ansprüche 1 bis 6, in dem die Bisphenol-Verbindung einer der folgenden Formeln entspricht: und

8. Verfahren nach einem der Ansprüche 1 bis 7, in dem der Kuppler ein Kuppler der in der folgenden Tabelle angegebenen Struktur ist: worin die Gruppen (f), (c), (g) und (k) die in Anspruch 4 angegebene Bedeutung besitzen.

9. Verfahren nach einem der Ansprüche 1 bis 8, bei dem das photographische Material ein mehrfarbiges photographisches Element ist mit einem Träger, auf dem sich eine ein gelbes Farbstoffbild bildende Einheit befindet, mit mindestens einer blau-empfindlichen Silberhalogenidemulsionsschicht, der mindestens ein Kuppler und ein blockiertes Bis-Phenol wie in einem der Ansprüche 1 bis 8 definiert zugeordnet ist, sowie purpurrote und blaugrüne Farbstoffbilder bildende Einheiten mit mindestens einer grün- oder rot-empfindlichen Silberhalogenidemulsionsschicht, der mindestens ein ein purpurrotes Farbstoffbild bildender Kuppler beziehungsweise ein ein blaugrünes Farbstoffbild bildender Kuppler zugeordnet ist, aufweist.

## Revendications

1. Méthode pour augmenter la Dₘₐₓ et le gamma et pour diminuer la Dₘᵢₙ de l'image de colorant jaune formée dans un produit photographique photosensible en couleurs comprenant un support recouvert d'une couche d'émulsion aux halogénures d'argent, 85% des halogénures étant constitués par du chlorure, et qui contient dans cette couche d'émulsion ou dans une couche adjacente, un coupleur jaune comprenant un groupe ballast de formule générale : dans laquelle
L¹ est -NHSO₂, -SO₂NH-, -OCO-, -COO-, -OSO₂- ou -SO₂O-,
R¹ est un atome d'halogène ou un groupe alkyloxy de 1 à 4 atomes de carbone,
R² est un groupe alkyle, substitué ou non, ou un groupe aryle, substitué ou non, de taille et de configuration suffisantes pour rendre le coupleur non-diffusible dans le produit photographique, et
X est un atome d'halogène, un groupe qui se sépare au couplage aryle, aryloxy, arylthio ou un groupe hétérocyclique,
le produit étant exposé et développé avec un procédé de traitement en couleurs comprenant une étape de développement chromogène en l'absence d'alcool benzylique, la méthode consistant à incorporer dans la couche contenant le coupleur, un dérivé du bisphénol comprenant deux cycles phénol liés, un des groupes hydroxy phénoliques étant substitué par un groupe bloquant et au moins un des cycles phénol étant substitué.

2. Méthode selon la revendication 1, dans laquelle le groupe R² comprend un groupe :

3. Méthode selon la revendication 1 ou 2 dans laquelle R¹ est un groupe chloro ou méthoxy.

4. Méthode selon l'une quelconque des revendications 1 à 3 dans laquelle le groupe X qui se sépare au couplage est l'un des groupes suivants :
(a)
(b)
(c)
(d)
(e)
(f)
(g) ou
(h)
(i)
(j)
-Cl
(k)

5. Méthode selon l'une quelconque des revendications 1 à 4 dans laquelle le dérivé du bisphénol a la formule : dans laquelle
A est un groupe bloquant tel qu'un groupe alkyle, par exemple, méthyle, éthyle, propyle ou butyle ; un groupe cycloalkyle, par exemple, cyclohexyle, alkényle ; un groupe aryle, par exemple, phényle ; un groupe acyle par exemple acétyle ou benzoyle ; un groupe alkylsulfonyle ou un groupe arylsulfonyle ;
L est une simple liaison ou un groupe de liaison tel qu'un groupe alkylène, par exemple, méthylène ; un groupe alkylidène, par exemple, butylidène ou 3,5,5,-triméthylhexylidène ; un hétéroatome, par exemple, un atome d'oxygène ou de soufre ; ou un groupe sulfonyle ; et
chaque R est, indépendamment un ou plusieurs substituants choisis chacun séparément parmi les groupes alkyle, alkoxy, alkényle, cycloalkyle ou aryle;
ou chaque R, indépendamment, représente les atomes nécessaires pour former, avec le cycle benzénique sur lequel il est attaché, une structure polycyclique aromatique condensée ;
tous les groupes alkyles, cycloalkyles, alkylène, alkényle, acyle et aryle mentionnés ci-dessus pouvant être substitués.

6. Méthode selon l'une quelconque des revendications 1 à 5, dans laquelle le dérivé du bisphénol a la formule générale : dans laquelle
A et L sont tels que définis dans la revendication 5 ; et
R³, R⁴, R⁵ et R⁶ sont chacun séparément des groupes alkyle, alkényle, cycloalkyle ou aryle, substitués ou non. De préférence, R³ et R⁴ sont identiques et R⁵ et R⁶ sont identiques,
les bisphénols d'alkylidène représentent un groupe préféré de stabilisateurs dans lequel le groupe de liaison L peut être -(CR⁷R⁸)ₙ- dans lequel R⁷ et R⁸ sont chacun séparément un atome d'hydrogène ou, éventuellement un groupe aryle, alkényle, cycloalkyle ou alkyle, substitué ou non, et n est un nombre entier compris entre 1 et 10, de préférence entre 1 et 3, préférablement 1.

7. Méthode selon l'une quelconque des revendications 1 à 6 dans laquelle le composé bisphénol a une des formules suivantes : et

8. Méthode selon l'une quelconque des revendications 1 à 7, dans laquelle le coupleur est un de ceux décrits dans le tableau suivant : dans lequel les groupes (f), (c), (g) et (k) sont tels que définis dans la revendication 4.

9. Méthode selon l'une quelconque des revendications 1 à 8, dans laquelle le produit photographique est un produit photographique en couleurs comprenant un support recouvert d'une zone formatrice de colorant jaune constituée d'au moins une couche d'émulsion aux halogénures d'argent sensible au bleu associée à au moins un coupleur et un composé bisphénol bloqué tel que défini dans l'une quelconque des revendications 1 à 8 et des zones formatrices d'image de colorant magenta et cyan comprenant au moins une couche d'émulsion aux halogénures d'argent sensibles au vert ou au rouge associée à au moins un coupleur formateur de colorant magenta, respectivement cyan.
